# EUROPEAN PATENT APPLICATION

(11) **EP 4 442 866 A1**
(43) Date of publication of application: **09.10.2024**
(21) Application number: 24168818.3
(22) Date of filing: 05.04.2024
(51) Int. Cl.: C25D 11/08, C25D 11/18

(54) **METHOD FOR MAKING A MANUFACTURED PRODUCT FOR WATCHMAKING, JEWELLERY, COSTUME JEWELLERY OR FOR THE PRODUCTION OF ACCESSORIES COMPRISING AN ALUMINIUM OXIDE LAYER AND MANUFACTURED PRODUCT SO OBTAINED**

(30) Priority: 06.04.2023 IT 202300006753
(71) Applicant: Patros S.r.l., 36066 Sandrigo (Vicenza) (IT)
(72) Inventor: BOTTENE, Diego, 36010 Monticello Conte Otto (Vicenza) (IT)
(74) Representative: Feltrinelli, Secondo Andrea

(57) **Abstract**

Method for the production of a manufactured product for watchmaking, jewellery, costume jewelery or for the production of accessories, comprising the steps of providing at least one base body substantially having the shape of the manufactured product (1) or at least part of it , wherein the base body is made of aluminium or an aluminium-based alloy and includes at least one external surface (2), subjecting the base body or at least part of the at least one external surface (2) to surface processing, subjecting the base body to anodic oxidation at low temperature, for example between 0°C and 15°C, for example hard anodic oxidation, obtaining the formation of a layer (3) of aluminium oxide, for example hard aluminium oxide, having a thickness (t) at the at least one part of the at least one external surface (2), wherein at least part of the layer (3) constitutes a visible and/or exposed surface of the manufactured product (1); manufactured product (1) comprising a layer (3) of aluminium oxide obtained by the method of the present invention.

## Description

### TECHNICAL FIELD OF THE INVENTION

The present invention refers to a method for the production of a manufactured product for watchmaking, jewellery, costume jewelery or for the production of accessories comprising a layer of aluminium oxide and the related manufactured product thus obtained.

### STATE OF THE PRIOR ART

Aluminium oxide is a ceramic oxide of aluminium. This material, apparently very fragile and not very usable, is instead fundamental in the industrial field, due to its properties such as resistance to acids, high thermal conductivity and poor electrical conductivity. It is used in many fields, such as the brick, refractory and ceramics industries, electronics and mechanics, and the biomedical industry.

Corundum is an aluminium oxide which generally can contain other elements such as iron, titanium, chromium, vanadium, etc.; it is a hard and stable mineral which, in addition to being present in nature, can also be produced artificially on an industrial level (synthetic mineral).

Furthermore, corundum has a very high density, which is unusual for a transparent mineral composed of elements with low atomic mass (oxygen and aluminium).

When it does not contain foreign elements, aluminium oxide is colourless (noble corundum); traces of different elements give the crystal different colours.

Corundum crystals are used in different applications, depending on the type and purity. For example, natural crystals are mainly used as precious stones, however artificial corundum gems are also very often used in jewellery.

In contrast, impure or substandard varieties are used industrially as abrasive materials. Hard anodic oxidation is a treatment performed on aluminium or its alloys and used in various sectors.

In particular, it is an electrochemical process that allows a compact layer of oxide, also called "hard aluminium oxide", to be obtained on the metal surface of the treated piece. This process uses electric current and its name derives from the fact that the piece or part to be treated is connected to the anode of an electrolytic cell.

It is therefore a surface treatment of aluminium that transforms the surface of the metal, or of the aluminium-based metal alloy, modifying its molecular structure. In fact, during the electrolytic process to which the aluminium is subjected, a patina or layer of oxide is formed which partly attaches to it.

This type of oxidation is carried out in the laboratory and has become a process applied in various industries, such as the mechanical, aeronautical, civil or military, automotive, etc. industries.

Application WO2006/056860 describes a method based on hard anodic oxidation applied to the jewelery or costume jewelery sector.

Application JPS57 104689 describes a method for manufacturing a product such as a watch which involves providing a layer of hard aluminium oxide and covering this layer with a fluoro-hydrocarbon based polymer.

Application EP3421646 describes a method for colouring an aluminium alloy element which involves forming a layer and covering this layer with a further metallic layer. Application US2008/274375 describes a method for producing coloured layers on a metal object.

Finally, application CN113106517 describes a method for preparing a ring equipped with a hardening layer and an overlying protective layer.

However, over the years, the need has arisen to prepare an implemented method which is easy and practical and which is able to give the products obtained improved properties in terms of resistance, as well as colour and/or in terms of mechanical characteristics, and/or elasticity.

### OBJECTS OF THE INVENTION

The aim of the present invention is to provide a method for the production of a manufactured product for watchmaking, jewellery, costume jewelery or for the production of accessories, for example fashion or design, comprising a layer of aluminium oxide, which is easy and practical to make.

Another object of the present invention is to provide a method for the production of a manufactured product for watchmaking, jewellery, costume jewelery or for the production of accessories, for example fashion or design, comprising a layer of aluminium oxide, which is capable of giving the resulting product certain characteristics in terms of appearance and/or colour.

A still further object of the present invention is to provide a method for the production of a manufactured product for watchmaking, jewellery, costume jewelery or for the production of accessories, for example fashion or design, comprising a layer of aluminum oxide, which is capable of giving the resulting product improved mechanical characteristics, for example in relation to the hardness and resistance of the product itself.

Furthermore, an object of the present invention is to provide a method for the production of a manufactured product for watchmaking, jewellery, costume jewelery or for the production of accessories, for example fashion or design, comprising a layer of aluminium oxide, which is capable of giving the resulting product hypoallergenic characteristics, i.e. which is capable of satisfactorily responding to the requirements required by the relevant regulations regarding precious metals or similar.

A still further object of the present invention is to provide a method whose costs are reduced.

In accordance with an aspect of the present invention, a method is provided for the production of a manufactured product for watchmaking, jewellery, costume jewelery or for the production of accessories, for example fashion or design, comprising a layer of aluminium oxide, according to claim 1.

In accordance with another aspect of the present invention, a manufactured product is provided for watchmaking, jewellery, costume jewelery or for the production of accessories, for example fashion or design, comprising a layer of aluminium oxide according to claim 12.

The dependent claims refer to preferred and advantageous forms of the invention.

### BRIEF DESCRIPTION OF THE DRAWINGS

Further characteristics and advantages of the present invention will be more evident from the detailed, non-exclusive description of a preferred embodiment example of a manufactured product according to the present invention, given by way of example, but not by way of limitation, in the attached drawing tables in which:
Figure 1 is a perspective view of a product manufactured according to the present invention, in the form of a ring in which a stone is set,
figure 2 is a perspective view of a product manufactured according to the present invention, in the form of a ring without setting,
figure 3 is a perspective view of a product manufactured according to the present invention, in the form of a buckle,
figure 4 is a perspective view of a product manufactured according to the present invention, in the form of a watch,
figure 5 represents a partial sectional view of a product manufactured according to the present invention,
figure 6 represents a detailed example of the view in figure 5.

### EMBODIMENTS OF THE INVENTION

The present invention refers to a manufactured product 1 for watchmaking (fig. 4), jewellery, costume jewelery (fig. 1 and 2) or for the creation of accessories (fig. 3), for example for fashion or design.

The manufactured product according to the invention has the shape of a bracelet, a ring, a necklace, a pendant, an earring, a brooch or a buckle for example of a watch or a belt, of an accessory for an item of clothing, for a shoe or for a bag, for a watch dial or part of it, etc.

The manufactured product 1 is made up of a base body substantially having the shape of the manufactured product 1 or at least of a part of it.

This bae body is made of aluminium, completely in aluminium or an aluminium-based alloy.

For example, the aluminium alloy may be an alloy of aluminium and zinc, known as Ergal or 7000 series alloy, or an alloy of aluminium, silicon, magnesium, and sometimes manganese, known as Anticorodal or 6000 series alloy.

The base body of the manufactured product 1, in at least one version of the present invention, is completely made of the material indicated above, i.e. aluminium or an aluminium-based alloy. This means that there are no layers of other metals or aluminium in a different degree of purity, compared to the total material of the base body itself. The base body includes at least one external surface 2 and a thickness S, constant or variable along the longitudinal or transversal extension of the manufactured product itself, depending on the specific shape or conformation of the latter.

The external surface 2 is for example the surface of the base body which is visible when the base body itself is made.

The manufactured product 1 also comprises at least one layer 3 of aluminium oxide, for example hard aluminium oxide. This at least one layer 3 is placed or applied or created on at least a part of the at least one external surface 2. In fact, therefore, the surface of the base body which is visible and/or exposed when the base body itself is made and/or in contact with the user, is made up of the at least one layer 3.

The base body and the layer 3 constitute a base structure of the manufactured product 1 on which pearls, stones and/or inserts can be applied, as better indicated below.

This layer 3 acts as a coating for the at least one part of the at least one external surface 2 involved. Therefore, in at least one part in which the layer 3 is present, the external surface 2 is no longer visible or exposed, since the layer 3 acts as the actual external surface.

The manufactured product 1 according to the present invention and/or its base body can be obtained in a single piece or by assembling two or more pieces or base bodies together.

The method according to the present invention first comprises a step of providing at least one base body of the manufactured product 1.

The base body can be made using one of the following processes: processing using machine tools such as for example lathe, milling machine, shearing machine and/or press, for example directly from a casting bar, forging for example from a bar, a plate or a die casting, moulding, CNC computerized numerical control processing, extrusion, casting, micro-casting or lost-wax micro-casting, for example which allows even complex geometries for the manufactured product 1, three-dimensional printing, additive manufacturing, for example - also in this case - for the obtaining of even complex geometries for the manufactured product 1, using a laser printer, for example marketed by Sisma SpA, a combination of the previous ones, etc.

In particular, according to an embodiment, the laser printer mentioned above, for example called "Mysint 100" or "Mysint 200" by Sisma, is a three-dimensional printer for the selective laser fusion of layers of metal powder. In detail, this printer has a small laser spot, compared to other printers, for example created by a fiber laser source, and this guarantees high quality and definition, even for the smallest details of the manufactured product 1. Furthermore, it is possible minimize the quantity of metal powder that constitutes the manufactured product in question, thanks to special measures. According to an embodiment, the laser spot of the three-dimensional printer has a diameter of between 50 and 60 micrometres, for example 55 micrometres or 30 micrometres if desired.

Furthermore, the materials printable with this printer can be precious metals such as gold, platinum, silver, or even bronze, and/or materials based on stainless steel, steel alloys, aluminium alloys, materials including titanium or other weldable metals. According to another embodiment, the three-dimensional laser printer can comprise a double laser system, possibly with appropriate calibration and in which the two lasers can optionally be overlapped.

The above laser printer may include a heating system, for example up to 200°C.

The basic body of the manufactured product 1 can therefore be subjected to one or more surface processes, such as: preparation (for example by means of a lathe or laser or other method) of at least one setting or setting seat for the subsequent setting of diamonds, pearls, precious stones, non-precious stones, polishing, of the manual or mechanical or automated type, for example machine polishing, engraving, for example with a burin or using special manual or automated tools, brightening, diamond cutting, colouring, application of pigments and/or dyes , setting of diamonds, pearls, precious stones, non-precious stones, etc., application or insertion of inserts made with metals other than aluminium, for example precious metals, such as gold, platinum, palladium, silver, or other materials such as titanium, carbon, metals in general, diamonds, natural and/or synthetic gems, etc, or a combination of the previous processes.

The method according to the present invention then includes a step of subjecting the base body, after having been made and possibly having been worked according to one or more of the surface processes indicated above, to anodic oxidation, for example preferably hard anodic oxidation.

This step includes the following sub-steps:
- connect the at least one base body of the manufactured product 1 to an anode of an electrolytic cell or tank,
- immerse at least part of the base body and/or at least part of the external surface 2 in an electrolytic cell or tank comprising an acidic electrolyte, such as for example sulfuric acid, possibly under agitation,
- pass an electric current, for example 3.5 A/dm² or less than 3.5 A/dm² or on average 3.5 A/dm², in said base body,
- obtain the formation of a layer 3 of aluminium oxide, for example of hard aluminium oxide, having a thickness t at at least one part of the at least one external surface 2.

The layer 3 originates directly from the material of the base body, at at least part of the at least one external surface 2 of the base body itself. This at least one part of the at least one external surface 2 is the one on which the layer 3 is desired to be created and/or obtained; therefore, it is that part that is subjected to anodic oxidation.

The layer 3 generally has a (natural) greyish colour, possibly dark, such as anthracite grey or tending towards black. In order to make the layer 3 take on a black and/or darker colour, it is possible to add at least one black pigmenting agent, such as for example black alumina, in powder form if desired, to the electrolytic cell or tank and/or to the acid electrolyte, in order to make the layer 3 to take on a black and/or darker colouring than (natural) grey and/or intense black colour.

In this way, since the black pigmenting agent is present while the layer 3 is being formed, it will be uniformly distributed within the layer 3 itself.

To connect the at least one base body of the manufactured product 1 to an anode of an electrolytic cell or tank, at least one support is used, capable of supporting, for example in a sort of scaffolding, even multiple base bodies simultaneously. Such at least one support may be in the form of a hook, perch, support frame, scaffold, etc. It has been seen that by making such at least one support in titanium, for example of grade 2, grade 3, grade 5, or higher, improved properties are obtained in the layer 3 resulting from the oxidation process.

In particular, it has been seen that, the more the titanium grade increases, and therefore the greater the hardness of the titanium used, the better is the quality of the resulting layer 3. According to a preferred version of the invention, therefore, the at least one support is made of grade 5 titanium.

In the event that the layer 3 is to be obtained only on a part or area of the manufactured product, the method can include a step of covering the part of the external surface 2 which must not be affected by the formation of the layer 3, so that, even if the entire base body is immersed in the electrolytic cell or tank, the layer 3 will be deposited only where desired. Naturally, this covering step must be carried out in such a way that the acidic electrolyte does not penetrate into the covered area, so as to precisely define the peripheral edges of layer 3 and in fact the demarcation between the area affected by the layer 3 and the part of the surface 2 in which this layer 3 is not deposited.

A peculiar characteristic of this step is that it occurs at a certain temperature, i.e. at a low temperature. By low temperature we mean a temperature lower than 15°C or preferably lower than 10°C or even more preferably equal to about 0°C or between 0°C and 15°C. For example, the electrolyte cell or tank is maintained at such a temperature, and/or the acidic electrolyte is maintained at such a temperature, and/or the surrounding environment is also maintained at such a temperature.

The immerging step lasts from a minimum of 20 minutes to a maximum of 6-7 hours, preferably between 30 minutes and 2 hours, even more preferably between 30 minutes to 1 hour or even more preferably between 40 minutes and 60-80 minutes. Based on the shorter or longer immersion time, a smaller or larger thickness t of the aluminium oxide layer 3 can be obtained.

Thanks to the low temperature at which the anionic oxidation step takes place, it is possible that the manufactured product 1 includes - before this electrolytic treatment - diamonds, pearls, precious stones or non-precious stones already set, inserts of a precious metal or other type, without that the treatment itself may damage these elements. In this way there is the advantage of not having to carry out setting operations after oxidation, obtaining a manufactured product substantially ready for use or sale. According to at least one version of the present invention, the anionic oxidation step occurs in accordance with the UNI 7796 standard.

There is therefore a step of extraction of the manufactured product 1 including the layer 3 from the electrolytic cell or tank and its detachment from the anode to which it is fixed. One or more subsequent processes can therefore follow such as: preparation of at least one setting or setting seat for setting diamonds, pearls, precious stones, non-precious stones, polishing, of the manual or mechanical or automated type, for example polishing by machine, engraving, for example with a burin or using special manual or automated tools, polishing, diamond cutting, colouring, application of pigments and/or dyes, setting of diamonds, pearls, precious stones, non-precious stones, chiseling, sandblasting, application or insertion of inserts made with metals other than aluminium, for example precious metals, such as gold, platinum, palladium, silver, or other materials such as titanium, carbon, metals in general, diamonds, natural and/or synthetic gems, or a combination of processes themselves.

This application step can take place via welding or brazing on site or via gluing and/or mechanical interlocking, etc.

In any case, at least according to one version of the present invention, a part or most of the layer 3 remains visible or exposed, despite the presence of settings, treatments, inserts or other materials indicated above.

The surface processing and subsequent processing indicated can be carried out manually or using special machinery, possibly equipped with automation systems, robots, for example anthropomorphic robots, special machines, etc.

The step of obtaining a layer 3 of aluminium oxide includes the steps of forming and deposing the layer 3 of aluminium oxide at least externally to the base body of the manufactured product 1, i.e. at least externally to the at least one part of the at least one external surface 2.

According to an alternative version, the step of obtaining an aluminium oxide layer 3 can comprise the following steps: formation and deposition of an external portion 3a of the aluminium oxide layer 3 externally to the base body, i.e. externally to the at least a part of the at least one external surface 2 and, possibly, simultaneous or previous formation and deposition of an internal portion 3b of the aluminium oxide layer 3 inside the base body, i.e. inside the at least one part of the at least one external surface 2. Naturally, the external portion 3a and the entire portion 3b, when both are present, are corresponding, that is, they are present in the same affected portion of the at least one external surface 2.

In this case, the external portion 3a (or in any case the layer 3) includes an external surface 3c which will become, once the manufactured product 1 is finished, the most external and/or visible and/or exposed surface thereof.

The aluminium oxide layer 3 is formed directly in contact with at least part of the external surface 2. Therefore, the aluminium oxide layer 3 is formed directly in contact with the material that constitutes the base body of the manufactured product 1.

In at least one version of the present invention, in fact, the manufactured product, after the anodic oxidation step, is made up exclusively of the material that constitutes the base body and the layer 3 of aluminium oxide (with the possibility of including pearls, stones, inserts, etc., which however do not constitute the base structure of the manufactured product, considering that the latter is made up only of the base body and layer 3 of aluminium oxide).

The characteristics of the aluminium oxide layer 3, or at least of its external surface 3c, are as follows:
- notable hardness, for example between 1100 and 1300 HV or between 50 and 1500 HV or between 50 and 1000 HV and compactness, which make the layer 3 a layer of protection for the manufactured product 1, and/or
- smooth and reflective and/or shiny aesthetic or external appearance; therefore, the external surface 3c is smooth and reflective and/or shiny, and/or
- possibility of being variously coloured or treated with coloured pigments or enamels or other colouring agents, such as for example a pigment or a black colour or another shade colour, etc.

These characteristics make it possible to obtain a manufactured product 1 of notable lightness and robustness, which can be worn comfortably and without the risk of breakage.

Furthermore, thanks to the properties of the aluminium oxide layer 3, the manufactured product has anti-scratch and impact-resistant properties. Similarly, the maintenance of the manufactured product is reduced to a minimum, being naturally shiny and free of dents and/or scratches caused by use.

The method according to the present invention also includes a step of tempering the aluminium oxide layer 3, and/or the manufactured product and/or the base body, in order to give greater hardness to the finished manufactured product.

The tempering step takes place in an oven, for example in a tunnel oven, in a hardening oven, in a thermal cycling oven, in a static oven, in a combination of the same, etc. The tempering step takes place at a temperature of 350°C or lower, or between 100°C and 350°C or between 150°C and 350°C or between 200°C and 350°C or between 250°C and 350° C.

In a version of the invention, during the takes place tempering step there may be a step of introducing nitrogen gas into the area where the tempering step takes place, for example in a static oven or in one of the ovens indicated above, possibly mixed with compressed air, if desired through automatic mixing using a control unit, in order to eliminate most of the impurities, deoxidize and/or remove any surface coatings present on and/or in the layer 3. In this way, a manufactured product and/or a base body is obtained, tempered and equipped with a layer 3 which does not release particles and/or patinas and/or which does not have impurities, therefore being perfectly tolerable for being worn and/or hypoallergenic. Furthermore, in this way, the layer 3 is not eroded or damaged and instead remains substantially unchanged both over time and in any subsequent processing.

In one version of the invention, the method according to the present invention may comprise a (further) deoxidation step which improves the quality of the resulting product. This deoxidation step can be carried out before or after the anodic oxidation and/or can be contemporaneous with the tempering step just described.

The deoxidation step can take place in an oven, for example in a tunnel oven, in a hardening oven, in a thermal cycling oven, in a static oven, in a combination thereof, etc., at a temperature of up to 150 °C or up to 200°C or up to 350°C or up to 450°C or less than 500°C and/or more than 50°C. This temperature is however lower than the melting temperature of the material that constitutes the manufactured product 1, for example at least 50-100°C lower than the melting temperature of the material that constitutes the manufactured product 1.

The method according to the present invention can also include a step of bringing the manufactured product or the base body to size, before or after the electrolytic treatment step. This step of bringing to size takes place for example in an oven, for example one of the ovens indicated above for other treatments. The result for the manufactured product is to become more ductile and malleable and therefore more easily workable. Therefore, by indicating that the step is related to "bringing the piece to size", it can also be understood in general as a step to facilitate the processing to which the base body or the manufactured product must be subjected.

Therefore, the method can include this step of bringing to size or facilitating the workability of the manufactured product or of the base body, subjecting this piece to a heat treatment, if desired at a temperature lower than 350°C which can be corresponding to or additional to the tempering step indicated above.

The layer 3 has a thickness of between 1 micron and 300 microns or between 20 microns and 200 microns or between 50 microns and 100 microns or 10 microns or 100 microns or 120 microns or 150 microns.

Furthermore, the external portion 3a and the internal portion 3b of the layer 3 can each have a thickness between 1 micron and 150 microns or between 10 microns and 100 microns or 60 microns or 50 microns or 30 microns.

According to a version of the present invention, the thickness t of the layer 3 is divided equally between the external portion 3a and the internal portion 3b (50% and 50%). According to a further version of the present invention, the thickness of the internal portion 3b represents:
- 30% of the total thickness t while the external portion 3a represents 70% of the total thickness to
- a percentage between 10% and 90%, or
- a percentage between 5% and 50%, or
- a percentage between 25% and 50%.

In at least one version of the present invention, the greater the thickness of the external portion 3a, the lower is the overall hardness of the aluminium oxide layer 3.

Going into more detail, the thickness of the internal portion 3b depends on the residence time of the manufactured product in the treatment tank. For example, a treatment or immersion time between 30 min and 80 min, in at least one version of the present invention, allows obtaining a thickness percentage relating to the internal portion 3b of approximately 30% or approximately 50% of the thickness total t of layer 3.

Since the internal portion 3b of aluminium oxide is positioned inside the external surface 2 of the manufactured product, a sort of step of absorption, by the material that makes up the base body, of the aluminium oxide caused by anionic oxidation treatment, takes place during the immersion step. For this reason, a longer immersion duration determines, in at least one version of the invention, a greater absorption of aluminium oxide and therefore a greater thickness of the internal portion 3b of the layer 3.

After the creation of the aluminium oxide layer 3, one or more subsequent processes can therefore be carried out, among those listed above.

Finally, there may be a final polishing step of the manufactured product 1 thus obtained. It has thus been seen that the invention presents the advantages indicated above.

The invention and the method thus conceived are susceptible to numerous modifications and variations, all falling within the scope of the inventive concept described in the present discussion.

## Claims

1. Method for making a manufactured product for watchmaking, jewellery, costume jewelery or for the production of accessories, comprising the following steps:
supplying at least one base body of said manufactured product (1) having a shape substantially corresponding to that of said manufactured product (1) or at least of a part thereof, wherein said base body is made of aluminium or an alloy based on aluminium and includes at least one external surface (2),
subjecting said base body or at least part of said at least one external surface (2) to surface processing,
subjecting said base body to anodic oxidation, for example hard anodic oxidation,
**characterized by the fact that** said step of subjecting said base body to anodic oxidation includes the following sub-steps:
- connecting said at least one base body to an anode of an electrolytic cell or tank, at a temperature, for example a low temperature, of about 0°C or lower than 10°C or lower than 15°C or between 0°C and 15°C,
- immersing at least part of said base body and/or said at least part of said at least one external surface (2) in an electrolytic cell or tank comprising an acidic electrolyte, such as for example sulfuric acid, possibly under agitation,
- passing an electric current, for example 3.5 A/dm² or less than 3.5 A/dm² or on average 3.5 A/dm², in said base body,
- obtaining the formation of a layer (3) of aluminium oxide, for example of hard aluminium oxide, having a thickness (t) at said at least part of said at least one external surface (2),
- tempering said layer (3) of aluminium oxide in an oven at a temperature of 350°C or lower,
- obtaining said manufactured product (1) comprising said layer (3), wherein at least part of said layer (3) constitutes a visible and/or exposed surface of said manufactured product (1).

2. Method according to claim 1, wherein said step of obtaining the formation of a layer (3) includes the following steps:
formation and deposition of said layer (3) of aluminium oxide at least externally to said at least one part of said at least one external surface (2), and/or
formation and deposition of an external portion (3a) of said layer (3) of aluminium oxide externally to said at least one part of said at least one external surface (2) and
simultaneous or previous formation and deposition of an internal portion (3b) of said layer (3) of aluminium oxide internally to said at least one part of said at least one external surface (2).

3. Method according to claim 1, wherein said immersing step lasts from a minimum of 20 minutes to a maximum of 6-7 hours, or between 30 minutes and 2 hours, or between 30 min to 1 hour or between 40 min and 60- 80 minutes, and possibly wherein said method comprises a step of extracting said manufactured product (1) including said layer (3) from said electrolytic cell or tank and a step of detaching said manufactured product (1) from the anode to which it is fixed.

4. Method according to any one of the previous claims, comprising a step of adding, in said electrolytic cell or tank and/or in said acidic electrolyte, at least one black pigmenting agent, such as for example black alumina, if desired in powder form, so as that said layer (3) assumes a black colouring and/or a colour darker than grey and/or an intense black colour, such that said black pigmenting agent is uniformly distributed within said layer (3) and/or wherein said step of connecting said at least one base body of said manufactured product (1) to said anode of said electrolytic cell or tank comprises providing at least one support, suitable for supporting, for example in a sort of scaffolding, at least one said base body, wherein said at least one support is made in titanium, such as for example of grade 2, grade 3, grade 5, or higher.

5. Method according to any one of the preceding claims, wherein said step of obtaining the formation of a layer (3) of aluminium oxide comprises forming a layer (3) having a thickness (t) between 1 micron and 300 microns or between 20 microns and 200 microns or between 50 microns and 100 microns or 10 microns or 100 microns or 120 microns or 150 microns and/or wherein said step of obtaining the formation of a layer (3) of aluminium oxide comprises forming said external portion (3a) and/or said internal portion (3b) of said layer (3) with a thickness between 1 micron and 150 microns or between 10 microns and 100 microns or 60 microns or 50 microns or 30 microns and/or wherein said internal portion (3b) has a thickness corresponding to 30% of said thickness (t), 50% of said thickness (t), between 10% and 90%, or between 5% and 50%, or between 25% and 50% of said thickness (t).

6. Method according to any of the previous claims, wherein said at least one surface processing includes: preparation by means of a lathe or laser or other method of at least one setting or setting seat for the subsequent setting of diamonds, pearls, precious stones, non-precious stones, polishing, of the manual or mechanical or automated type, for example machine polishing, engraving, for example with a burin or using special manual or automated instruments, brightening, diamond-cutting, colouring, application of pigments and/or dyes, setting of diamonds, pearls, stones precious, non-precious stones, etc., application or insertion of inserts made with metals other than aluminium, for example precious metals, such as gold, platinum, palladium, silver, or other materials such as titanium, carbon, metals in general, diamonds, natural and/or synthetic gems, etc. or a combination of the previous processes.

7. Method according to any of the previous claims, wherein said manufactured product (1) comprising said layer (3) is subjected to one or more subsequent processes such as for example: provision of at least one setting or setting seat for setting diamonds, pearls, precious stones, non-precious stones, polishing, of the manual or mechanical or automated type, for example machine polishing, engraving, for example with a burin or using special manual or automated tools, brightening, diamond cutting, colouring, application of pigments and/or or dyes, setting diamonds, pearls, precious stones, non-precious stones, chasing, sandblasting, application or insertion of inserts made with metals other than aluminium, for example precious metals, such as gold, platinum, palladium, silver, or other materials such as titanium, carbon, metals in general, diamonds, natural and/or synthetic gems, or a combination of the processes themselves.

8. Method according to any one of claims 6 or 7, wherein said application step occurs via welding or brazing on site or via gluing and/or mechanical interlocking, etc.

9. Method according to any of the preceding claims, wherein said step of providing said base body comprises providing an alloy of aluminium and zinc, known as Ergal or 7000 series alloy, or an alloy of aluminium, silicon, magnesium and sometimes manganese, known as an Anticorodal or 6000 series alloy.

10. Method according to any of the previous claims, wherein said step of providing said base body comprises producing said base body by one of the following processes: processing by machine tools such as for example lathe, milling machine, shearing machine and/or press, for example directly from a casting bar, forging for example from a bar, a plate or a die casting, moulding, CNC computerized numerical control machining, extrusion, casting, micro-casting or lost wax micro-casting, for example which allows even complex geometries for the manufactured product (1), three-dimensional printing, additive manufacturing, for example to obtain even complex geometries for the manufactured product (1), using a laser printer, a combination of the previous ones, etc.

11. Method according to any of the previous claims, comprising at least one of the following steps:
- wherein said tempering step occurs in a tunnel oven, in a hardening oven, in a thermal cycling oven, in a static oven, in a combination thereof, etc., and/or
- wherein said tempering step occurs at a temperature between 100°C and 350°C or between 150°C and 350°C or between 200°C and 350°C or between 250°C and 350°C, and/or
- wherein during said tempering step there occurs a step of introducing into the area where said tempering step takes place, for example in a tunnel oven, in a hardening oven, in an oven with thermal cycles, in a static oven, in a combination of the same, nitrogen gas, possibly mixed with compressed air, if desired through automatic mixing using a control unit, in order to eliminate most of the impurities, deoxidize and/or remove any surface coatings present on and/or in said layer ( 3), and/or
- deoxidize said layer (3) of aluminium oxide, said manufactured product (1) or said base body in an oven, in a tunnel oven, in a hardening oven, in an oven with thermal cycles, in a static oven , in a combination thereof, etc., at a temperature up to 150°C or up to 200°C or up to 350°C or up to 450°C or below 500°C,
- bringing to size or facilitate the workability of said manufactured product (1) or said base body, by subjecting said base body or said manufactured product (1) to a heat treatment in an oven, in a tunnel oven, in a with thermal cycles, in a static oven, in a combination of the same, etc.

12. Manufactured product for watchmaking, jewellery, costume jewelery or for the production of accessories, obtainable with a method according to one or more of claims 1 to 11, wherein said manufactured product (1) comprises at least one base body having a shape substantially corresponding to that of said manufactured product (1) or at least one part thereof, wherein said base body is made of aluminium or an aluminium-based alloy and includes at least one external surface (2), **characterized by the fact that** at least part of said base body and/or at least part of said at least one external surface (2) comprises a layer (3) of aluminium oxide, for example of hard aluminium oxide, having a thickness (t), wherein at least part of said layer (3) constitutes a visible and/or exposed surface of said manufactured product (1).

13. Manufactured product according to claim 12, wherein said layer (3) comprises an external portion (3a) of said layer (3) of aluminium oxide placed externally in and in contact with said at least one part of said at least one external surface (2) and an internal portion (3b) of said layer (3) of aluminium oxide placed internally in contact with said at least one part of said at least one external surface (2), wherein said external portion (3a) is placed at said internal portion (3b) and constitutes said visible and/or exposed surface of said manufactured product (1).

14. Manufactured product according to claim 12 or 13, wherein said thickness (t) is between 1 micron and 300 microns or between 20 microns and 200 microns or between 50 microns and 100 microns or 10 microns or 100 microns or 120 microns or 150 microns and/or wherein said external portion (3a) and/or said internal portion (3b) of said layer (3) has a thickness of between 1 micron and 150 microns or between 10 microns and 100 microns or 60 microns or 50 microns or of 30 microns and/or wherein said internal portion (3b) has a thickness corresponding to 30% of said thickness (t), 50% of said thickness (t), between 10% and 90%, or between 5% and 50%, or between 25% and 50% of said thickness (t).

15. Manufactured product according to any of claims 12 to 14, comprising at least one setting or setting seat for at least one of diamonds, pearls, precious stones, non-precious stones, an engraving, for example with a burin or using special manual or automated tools, a polishing, a diamond finishing, a colouring , pigments and/or dyes, at least one insert made with metals other than aluminium, for example precious metals, such as gold, platinum, palladium, silver, or other materials such as titanium, carbon, metals in general, diamonds, natural and/or or synthetic gems, etc. or a combination thereof.

16. Manufactured product according to any of claims 12 to 15, wherein said layer (3) has an external surface (3c) which is shiny, and/or sparkling and/or smooth, and/or reflective, and/or coloured or treated with coloured pigments or enamels or other colouring agents, and/or wherein said base body comprises an alloy of aluminium and zinc, known as Ergal alloy or of the 7000 series, or an alloy of aluminium, silicon, magnesium and, if desired, manganese, known as Anticorodal alloy or of the 6000 series, and/or or wherein said layer (3) is a hypoallergenic layer, for example as it is free of impurities and risks of releasing particles when in contact with a user.
